

Feb. 16, 1937.

P. VOEGELI-JAGGI

2,070,734

PROCESS OF MANUFACTURING GRINDING TOOLS

Original Filed May 15, 1934

Fig. 1



Fig. 2



Fig. 3



Inventor:

Philip Voegeli-Jaggi

By *Paul Voegeli*  
Attorney

## UNITED STATES PATENT OFFICE

2,070,734

PROCESS OF MANUFACTURING GRIND-  
ING TOOLS

Philipp Voegeli-Jaggi, Bern, Switzerland

Substitute for application Serial No. 725,795, May  
15, 1934. This application February 19, 1936,  
Serial No. 64,782. In Switzerland April 27,  
1934

12 Claims. (Cl. 51—280)

The present invention relates to a type of abrasive article and to a method of manufacturing the same. The invention relates more particularly to an abrasive body containing diamonds embedded in a mass of heat-hardened artificial resin associated with fillers.

This application is a substitute for my pending United States application, Serial No. 725,795, filed May 15, 1934.

10 Diamond wheels have been used, for example, in making, cutting or grinding tools for working on hard alloys. In the use of such wheels it is found that the diamond particles do not wear out by diminution in size of the abrasive particles on the working surface in the same manner as when softer abrasive particles are used, such as fused alumina or silicon carbide. When abrasive wheels, containing particles of the last-mentioned materials are used, it is necessary that the bond 15 should be of such a character that a worn abrasive particle can be released from the bond and the work of grinding taken up by a fresh adjacent particle. On account of the greater hardness of diamond particles, on the other hand, it is desirable that a diamond particle should be held on the working surface as long as possible.

Difficulties have been encountered in holding diamond particles against the stress of grinding when various kinds of artificial resin (associated, 20 for example, with a graphite filler) have been used as bonding materials.

In accordance with the present invention it has been found that an improvement in the grinding efficiency of diamond wheels was obtained when 25 an artificial resin bonding material was mixed with ferric oxide and charcoal in addition to the graphite mentioned above. I have found the variety of ferric oxide known as English red or colcothar suitable for the present purpose. The 30 bond formed by mixing ferric oxide with graphite and a synthetic resin and subsequently curing the resin is very hard. Embedded in this mass, the diamond particles resist for a very long time the mechanical stress of grinding. The durability 35 and therefore the economy effected in the use of diamond wheels of this type is therefore increased by making them in the manner indicated above and described in more detail below. A grinding tool made of the described mixture may be fixed 40 easily upon a base of artificial resin so that the grinding mass may be nearly all used. In certain cases the grinding tool may be mounted on a metallic base, but this is not absolutely necessary.

In the drawing:

55 Figure 1 is an axial sectional view of a grind-

ing wheel made in accordance with the present invention.

Fig. 2 is a similar view, showing a modified form of wheel.

Fig. 3 is another view similar to Fig. 1, showing a further modified form of wheel.

For making a grinding wheel of the type illustrated in Fig. 1, the following constituents are employed:

|                     | Parts |
|---------------------|-------|
| Pulverized charcoal | 10    |
| Graphite            | 50    |
| Colcothar           | 50    |
| Diamond powder      | 75    |
|                     | 26    |
|                     | 15    |

These constituents are thoroughly mixed with some pulverized artificial resin and a relatively much larger quantity of liquid phenol condensation product resin. The mixture is made at a temperature of about 212° F. When the mixture 20 has become a homogeneous paste, it is placed in a mold into which there has been previously introduced a compressed disc *a* of artificial resin. This disc is intended to form a support for the grinding portion *b*. The paste is pressed against 25 the artificial resin disc in a hot state. The portions of the paste adjacent the disc serve to unite the grinding body *b* with the disc *a* when the resin in both *b* and *a* are cured at a suitable temperature. The integral body thus formed can be 30 fixed on an iron support *c*.

Where coarser diamond particles are chosen, silicon carbide particles are used in quantities equal to those of the diamond particles. This softens the grinding effect.

The admixed colcothar or ferric oxide causes 35 not only a hardening of the whole mixture but is also readily incorporated with the resinous mass during the mixing operation. Its presence does not interfere with the curing of the resin. The adhesion of the bond on the diamond particles appears to be increased since greater grinding efficiency is obtained.

Another form of grinding wheel is shown in Fig. 2. The disc *a'* is formed of artificial resin 40 such as phenolic condensation product resin and is in the form of a hollow cylinder or disc. The complete wheel is disc-shaped.

In the third form of grinding wheel (illustrated in Fig. 3) the iron support *c* is disc-shaped.

The grinding portion is in the form of an annular resinous body *b'* which is united to the disc *a'* as indicated above by means of pressure and heat. The disc *a'* serves to attach the grinding element *b'* to the iron support *c'*.

The formula given above discloses a large proportion of charcoal associated with the resinous bond for diamond particles. It has been found that charcoal has a beneficial effect apart from iron oxide as indicated from results obtained with wheels A and B, whose constituents are given below, the constituents being given as per cent.

| 10 | Wheel | Diamonds | Secondary abrasive | Bond | Fillers cured resin | Charcoal |
|----|-------|----------|--------------------|------|---------------------|----------|
| 15 | A     | 10       | 22                 | 20   | 48                  | 0        |
|    | B     | 10       | 22                 | 20   | 38                  | 10       |

The wheel B differed principally from the wheel A in that part of the fillers was replaced by charcoal in an amount sufficient to illustrate the valuable characteristics imparted by it. The grinding efficiency of wheel B was nearly twice as great as that of wheel A. Neither wheel A nor wheel B contained substantial amounts of iron oxide. The cutting rate of the wheel containing charcoal was also considerably greater than that of the wheel that did not contain charcoal.

I claim:

1. A process of making abrasive bodies, comprising mixing together approximately by weight 50 parts of pulverized charcoal, 50 parts of graphite, 75 parts of ferric oxide, 26 parts of diamond powder, some powdered artificial resin and a relatively large quantity of liquid artificial resin, heating the mixture to about 212° F. to form a homogeneous paste, introducing the paste into a mold, and subjecting the same to pressure while hot to form a unitary body.
2. A grinding body comprising diamond parti-

cles, graphite and ferric oxide bonded into a unitary mass by an artificial resin.

3. A grinding body comprising diamond particles, graphite, powdered charcoal and ferric oxide bonded into a unitary mass by an artificial resin.

4. A grinding body comprising abrasive grains, graphite, powdered charcoal and ferric oxide bonded into a unitary body by an artificial resin.

5. A grinding body comprising approximately 10 by weight 50 parts of pulverized charcoal, 50 parts of graphite, 75 parts of ferric oxide and 26 parts of diamond powder bonded together by an artificial resin.

6. A grinding body comprising diamond particles, graphite and colcothar bonded into a unitary mass by an artificial resin.

7. A grinding body comprising approximately by weight 50 parts of pulverized charcoal, 50 parts of graphite, 75 parts of colcothar and 26 parts of diamond powder bonded together by an artificial resin.

8. A grinding body comprising diamond particles and powdered charcoal bonded into a unitary mass by an artificial resin.

9. A grinding body comprising abrasive grains and powdered charcoal bonded into a unitary mass by an artificial resin.

10. A grinding body comprising diamonds and powdered charcoal bonded into a unitary mass 30 by an artificial resin.

11. A grinding body comprising diamond particles, graphite, and powdered charcoal bonded into a unitary mass by an artificial resin.

12. A grinding body comprising diamond particles, ferric oxide, and powdered charcoal bonded into a unitary mass by an artificial resin.

PHILIPP VOEGLI-JAGGI.